



US006193839B1

(12) **United States Patent**  
Ampulski et al.

(10) **Patent No.:** US 6,193,839 B1  
(45) **Date of Patent:** \*Feb. 27, 2001

(54) **METHOD OF MAKING WET PRESSED TISSUE PAPER WITH FELTS HAVING SELECTED PERMEABILITIES**

(75) Inventors: **Robert Stanley Ampulski**, Fairfield; **Ward William Ostendorf**, West Chester, both of OH (US)

(73) Assignee: **The Procter & Gamble Company**, Cincinnati, OH (US)

(\*) Notice: This patent issued on a continued prosecution application filed under 37 CFR 1.53(d), and is subject to the twenty year patent term provisions of 35 U.S.C. 154(a)(2).

Subject to any disclaimer, the term of this patent is extended or adjusted under 35 U.S.C. 154(b) by 0 days.

(21) Appl. No.: **08/928,388**

(22) Filed: **Sep. 12, 1997**

**Related U.S. Application Data**

(60) Division of application No. 08/672,293, filed on Jun. 28, 1996, now Pat. No. 5,776,307, which is a continuation-in-part of application No. 08/460,949, filed on Jun. 5, 1995, now abandoned, which is a continuation-in-part of application No. 08/358,661, filed on Dec. 19, 1994, now Pat. No. 5,637,194, which is a continuation-in-part of application No. 08/170,140, filed on Dec. 20, 1993, now abandoned.

(51) **Int. Cl.** <sup>7</sup> **D21F 11/00**

(52) **U.S. Cl.** **162/117; 162/205**

(58) **Field of Search** ..... 162/111, 117, 162/109, 205, 358.1, 361, 362; 264/284, 293, 324

(56) **References Cited**

U.S. PATENT DOCUMENTS

3,537,954 \* 11/1970 Justus .

FOREIGN PATENT DOCUMENTS

2901743 \* 8/1979 (DE) ..... 162/358.2  
297736 \* 3/1971 (SU) ..... 162/358.2

\* cited by examiner

*Primary Examiner*—Brenda A. Lamb

(74) *Attorney, Agent, or Firm*—Vladimir Vitenberg; Larry L. Huston; Gerry S. Gressel

(57) **ABSTRACT**

The present invention provides method for making a wet pressed paper web. An embryonic web of papermaking fibers is formed on a foraminous forming member, and transferred to an imprinting member to deflect a portion of the papermaking fibers in the embryonic web into deflection conduits in the imprinting member. The web and the imprinting member are then pressed between first and second dewatering felts in a compression nip to further deflect the papermaking fibers into the deflection conduits in the imprinting member and to remove water from both sides of the web. The first felt is positioned adjacent a first surface of the web. The imprinting member is positioned between the second surface of the web and the second felt. The second felt has an air permeability which can be greater than that of the first felt.

**10 Claims, 7 Drawing Sheets**





Fig. 1



Fig. 2



Fig. 3



Fig. 4



Fig. 5



Fig. 6



Fig. 7



Fig. 8





Fig. 10



Fig. 11



Fig. 12

**METHOD OF MAKING WET PRESSED  
TISSUE PAPER WITH FELTS HAVING  
SELECTED PERMEABILITIES**

This is a divisional of application Ser. No. 08/672,293, filed on Jun. 28, 1996 now U.S. Pat. No. 5,776,307 which is a continuation-in-part of application Ser. No. 08/460,949 filed Jun. 5, 1995 now abandoned, which is a continuation-in-part of application Ser. No. 08/358,661 filed Dec. 19, 1994 now U.S. Pat. No. 5,637,194 which is a continuation-in-part of Ser. No. 08/170,140 filed Dec. 20, 1993 now abandoned.

**FIELD OF THE INVENTION**

The present invention is related to papermaking, and more particularly, to a method for making a wet pressed tissue paper web.

**BACKGROUND OF THE INVENTION**

Disposable products such as facial tissue, sanitary tissue, paper towels, and the like are typically made from one or more webs of paper. If the products are to perform their intended tasks, the paper webs from which they are formed must exhibit certain physical characteristics. Among the more important of these characteristics are strength, softness, and absorbency. Strength is the ability of a paper web to retain its physical integrity during use. Softness is the pleasing tactile sensation the user perceives as the user crumples the paper in his or her hand and contacts various portions of his or her anatomy with the paper web. Softness generally increases as the paper web stiffness decreases. Absorbency is the characteristic of the paper web which allows it to take up and retain fluids. Typically, the softness and/or absorbency of a paper web is increased at the expense of the strength of the paper web. Accordingly, papermaking methods have been developed in an attempt to provide soft and absorbent paper webs having desirable strength characteristics.

U.S. Pat. No. 3,301,746 issued to Sanford et al. discloses a paper web which is thermally pre-dried with a through air-drying system. Portions of the web are then impacted with a fabric knuckle pattern at the dryer drum. While the process of Sanford et al. is directed to providing improved softness and absorbency without sacrificing tensile strength, water removal using the through-air dryers of Sanford et al. is very energy intensive, and therefore expensive.

U.S. Pat. No. 3,537,954 issued to Justus discloses a web formed between an upper fabric and a lower forming wire. A pattern is imparted to the web at a nip where the web is sandwiched between the fabric and a relatively soft and resilient papermaking felt. U.S. Pat. No. 4,309,246 issued to Hulit et al. discloses delivering an uncompacted wet web to an open mesh imprinting fabric formed of woven elements, and pressing the web between a papermaker's felt and the imprinting fabric in a first press nip. The web is then carried by the imprinting fabric from the first press nip to a second press nip at a drying drum. U.S. Pat. No. 4,144,124 issued to Turunen et al. discloses a paper machine having a twin-wire former having a pair of endless fabrics, which can be felts. One of the endless fabrics carries a paper web to a press section. The press section can include the endless fabric which carries the paper web to the press section, an additional endless fabric which can be a felt, and a wire for pattern embossing the web.

Both Justus and Hulit et al. suffer from the disadvantage that they press a wet web in a nip having only one felt.

During pressing of the web, water will exit both sides of the web. Accordingly, water exiting the surface of the web which is not in contact with a felt can re-enter the web at the exit of the press nip. Such re-wetting of the web at the exit of the press nip reduces the water removal capability of the press arrangement, disrupts fiber-to-fiber bonds formed during pressing, and can result in rebulking of the portions of the web which are densified in the press nip.

Turunen et al. discloses a press nip which includes two endless fabrics, which can be felts, and an imprinting wire. However, Turunen et al. does not transfer the web from a forming wire to an imprinting fabric to provide initial deflection of portions of the wet web into the imprinting fabric prior to pressing the web in the press nip. The web in Turunen can therefore be generally monoplanar at the entrance to the press nip, resulting in overall compaction of the web in the press nip. Overall compaction of the web is undesirable because it limits the difference in density between different portions of the web by increasing the density of relatively low density portions of the web.

In addition, Hulit et al., and Turunen et al. provide press arrangements wherein the imprinting fabric has discrete compaction knuckles, such as at the warp and weft crossover points of woven filaments. Discrete compacted sites do not provide a wet molded sheet having a continuous high density region for carrying loads and discrete low density regions for providing absorbency.

Embossing can also be used to impart bulk to a web. However, embossing of a dried web can result in disruption of bonds between fibers in the web. This disruption occurs because the bonds are formed and then set upon drying of the web. After the web is dried, moving fibers normal to the plane of the web disrupts fiber to fiber bonds, which in turn results in a web having less tensile strength than existed before embossing.

In conventional pressed papermaking operations employing two felts, the paper web is positioned between two felts. One side of the paper web is in contact with one of the felts, and the other side of the paper web is in contact with the other felt. At the exit of the nip, the paper web follows one of the felts. The other felt is separated from the paper web. It is important that the web follow the intended felt, so that the web is directed to the appropriate downstream operations.

To ensure the web follows the intended felt, conventional pressed papermaking operations use two felts having different structures. The felt which is intended to carry the paper web from the nip has a finer, more dense construction than the felt which is to be separated from the web at the nip exit. The felt having a finer, more dense construction is characterized by having a lower air permeability than the other felt. The finer, more dense construction of the felt carrying the paper web from the nip exit helps ensure that the web follows that felt, thereby avoiding unintentional transfer of the web to the other felt.

Paper scientists continue to search for improved paper structures that can be produced economically, and which provide increased strength without sacrificing softness and absorbency.

One object of the present invention is to provide a method for dewatering and molding a paper web.

Another object of the present invention is to press a web and an imprinting member between two felt layers, wherein one felt, which is in flow communication with conduits in the imprinting member, has a relatively high air permeability, and wherein the other felt, which is positioned adjacent a surface of the web, can have a relatively low air permeability.

Another object of the present invention is to provide a non-embossed patterned paper web having a relatively high density continuous network, and a plurality of relatively low density domes dispersed throughout the continuous network.

### SUMMARY OF THE INVENTION

The present invention provides a method for molding and dewatering a paper web. According to one embodiment of the present invention, an embryonic web of papermaking fibers is formed on a foraminous forming member, and transferred to an imprinting member having a web imprinting surface. The web can be transferred to the imprinting member to deflect a portion of the papermaking fibers in the embryonic web into a deflection conduit portion of the imprinting member without densifying the embryonic web. The web and the imprinting member are then positioned between first and second dewatering felt layers in a compression nip. In one embodiment, the imprinting member is a composite imprinting member having the web imprinting surface joined to the second felt layer.

The first felt layer is positioned adjacent a first face of the web in the nip. The imprinting surface of the imprinting member is positioned adjacent the second face of the web in the nip. The second felt layer is positioned in the nip to be in fluid communication with the deflection conduit portion of the imprinting member. The web is pressed in the compression nip to form a molded web.

The second felt layer has an air permeability of at least about 30 cubic feet per minute per square foot, and preferably at least about 40 cubic feet per minute per square foot. In one embodiment, the second felt layer has an air permeability which is between about 40 and about 120 cubic feet per minute per square foot.

The second felt layer can have an air permeability which is greater than the air permeability of the first felt layer. The second felt layer can have an air permeability which is at least about 1.5 times greater than the air permeability of the first felt layer. The relatively high permeability of the second felt layer allows water to be easily removed from the second felt layer both upstream and downstream of the compression nip, such as with one or more vacuum devices.

Removing water from the second felt layer upstream of the compression nip can help reduce the consistency of the web upstream of the nip. The reduced consistency upstream of the nip reduces the amount of water that must be removed by the nip for a given web consistency at the nip exit. The relatively high permeability of the second felt layer also allows water to be easily removed from the second felt layer downstream of the compression nip, thereby reducing rewet of the web.

At the nip exit, the first felt layer can be separated from the first face of the web, and carried on the imprinting member from the nip exit to the drying drum. The web can be pressed between the imprinting member and the drying drum, and then creped from the surface of the drum.

### BRIEF DESCRIPTION OF THE DRAWINGS

While the specification concludes with claims particularly pointing out and distinctly claiming the present invention, the invention will be better understood from the following description taken in conjunction with the accompanying drawings in which:

FIG. 1 is a schematic representation of one embodiment of a continuous papermaking machine illustrating transferring a paper web from a foraminous forming member to a

foraminous imprinting member, carrying the paper web on the foraminous imprinting member to a compression nip, and pressing the web carried on the foraminous imprinting member between first and second dewatering felts in the compression nip.

FIG. 2 is a schematic illustration of a plan view of a foraminous imprinting member having a first web contacting face comprising a macroscopically monoplanar, patterned continuous network web imprinting surface defining within the foraminous imprinting member a plurality of discrete, isolated, non connecting deflection conduits.

FIG. 3 is a cross-sectional view of a portion of the foraminous imprinting member shown in FIG. 2 as taken along line 3—3.

FIG. 4 is an enlarged schematic illustration of the compression nip shown in FIG. 1, showing a first dewatering felt positioned adjacent a first face of the web, the web contacting face of the foraminous imprinting member positioned adjacent the second face of the web, and a second dewatering felt positioned adjacent the second felt contacting face of the foraminous imprinting member, wherein the compression nip comprises opposed convex and concave compression surfaces.

FIG. 5 is a schematic illustration of a compression nip according to an alternative embodiment of the invention, wherein the paper web is positioned between a first dewatering felt and a composite imprinting member comprising a foraminous web patterning layer formed from a photopolymer joined to the surface of a second dewatering felt, and wherein the web, the first felt, and the composite imprinting member are positioned between opposed convex and concave compression surfaces in the compression nip.

FIG. 6 is a schematic illustration of a plan view of a molded paper web formed using the foraminous imprinting member of FIGS. 2 and 3.

FIG. 7 is a schematic cross-sectional illustration of the paper web of FIG. 6 taken along line 7—7 of FIG. 6.

FIG. 8 is an enlarged view of the cross-section of the paper web shown in FIG. 7.

FIG. 9 is an alternative embodiment of a paper machine according to the present invention using the compression nip configuration shown in FIG. 5 and having a composite imprinting member comprising a foraminous web patterning layer formed from a photopolymer joined to the surface of a dewatering felt layer.

FIG. 10 is a schematic illustration of a cross-section of a composite imprinting member.

FIG. 11 is a schematic illustration of a plan view of a foraminous imprinting member having a web contacting face comprising a continuous, patterned deflection conduit and a plurality of discrete, isolated web imprinting surfaces.

FIG. 12 is a schematic illustration of a plan view of a foraminous imprinting member having a semi-continuous web imprinting surface.

### DETAILED DESCRIPTION OF THE INVENTION

FIG. 1 illustrates one embodiment of a continuous papermaking machine which can be used in practicing the present invention. The process of the present invention comprises a number of steps or operations which occur in sequence. While the process of the present invention is preferably carried out in a continuous fashion, it will be understood that the present invention can comprise a batch operation, such as a handsheet making process. A preferred sequence of

steps will be described, with the understanding that the scope of the present invention is determined with reference to the appended claims.

According to one embodiment of the present invention, an embryonic web 120 of papermaking fibers is formed from an aqueous dispersion of papermaking fibers on a foraminous forming member 11. The embryonic web 120 is then transferred to a foraminous imprinting member 219 having a first web contacting face 220 comprising a web imprinting surface and a deflection conduit portion. A portion of the papermaking fibers in the embryonic web 120 are deflected into the deflection conduit portion of the foraminous imprinting member 219 without densifying the web, thereby forming an intermediate web 120A.

The intermediate web 120A is carried on the foraminous imprinting member 219 from the foraminous forming member 11 to a compression nip 300. The nip 300 can have a machine direction length of at least about 3.0 inches. The nip 300 has opposed compression surfaces. The opposed compression surfaces can be opposed convex and concave compression surfaces, with the convex compression surface being provided by a press roll 362 and the opposed concave compression surface being provided by a shoe press assembly 700. Alternatively, the nip 300 can be formed between two press rolls. In this case, the nip length can be less than 3.0 inches.

A first dewatering felt layer 320 is positioned adjacent the intermediate web 120A, and a second dewatering felt layer 360 is positioned adjacent the foraminous imprinting member 219. The second felt layer 360 has an air permeability of at least about 30 cubic feet per minute per square foot, and preferably at least about 40 cubic feet per minute per square foot. In one embodiment, the second felt layer 360 has an air permeability which is between about 40 and about 120 cubic feet per minute per square foot. The second felt layer 360 can have an air permeability which is greater than the air permeability of the first felt layer 320. The second felt layer can have an air permeability which is at least about 1.5 times greater than the air permeability of the first felt layer.

The intermediate web 120A and the foraminous imprinting member 219 are then pressed between the first and second dewatering felts 320 and 360 in the compression nip 300 to further deflect a portion of the papermaking fibers into the deflection conduit portion of the imprinting member 219; to density a portion of the intermediate web 120A associated with the web imprinting surface; and to further dewater the web by removing water from both sides of the web, thereby forming a molded web 120B which is relatively drier than the intermediate web 120A.

The molded web 120B is carried from the compression nip 300 on the foraminous imprinting member 219. The molded web 120B can be pre-dried in a through air dryer 400 by directing heated air to pass first through the molded web, and then through the foraminous imprinting member 219, thereby further drying the molded web 120B. The web imprinting surface of the foraminous imprinting member 219 can then be impressed into the molded web 120B such as at a nip formed between a roll 209 and a dryer drum 510, thereby forming an imprinted web 120C. Impressing the web imprinting surface into the molded web can further density the portions of the web associated with the web imprinting surface. The imprinted web 120C can then be dried on the dryer drum 510 and creped from the dryer drum by a doctor blade 524.

Examining the process steps according to the present invention in more detail, a first step in practicing the present

invention is providing an aqueous dispersion of papermaking fibers derived from wood pulp to form the embryonic web 120. The papermaking fibers utilized for the present invention will normally include fibers derived from wood pulp. Other cellulosic fibrous pulp fibers, such as cotton linters, bagasse, etc., can be utilized and are intended to be within the scope of this invention. Synthetic fibers, such as rayon, polyethylene and polypropylene fibers, may also be utilized in combination with natural cellulosic fiber. One exemplary polyethylene fiber which may be utilized is Pulpex™, available from Hercules, Inc. (Wilmington, Del.). Applicable wood pulps include chemical pulps, such as Kraft, sulfite, and sulfate pulps, as well as mechanical pulps including, for example, groundwood, thermomechanical pulp and chemically modified thermomechanical pulp. Pulps derived from both deciduous trees hereinafter, also referred to as "hardwood") and coniferous trees (hereinafter, also referred to as "softwood") may be utilized. Also applicable to the present invention are fibers derived from recycled paper, which may contain any or all of the above categories as well as other non-fibrous materials such as fillers and adhesives used to facilitate the original papermaking.

In addition to papermaking fibers, other components or materials may be added to the papermaking furnish. The types of additives desirable will be dependent upon the particular end use of the tissue sheet contemplated. For example, in products such as toilet paper, paper towels, facial tissues and other similar products, high wet strength is a desirable attribute. Thus, it is often desirable to add to the papermaking furnish chemical substances known in the art as "wet strength" resins.

A general dissertation on the types of wet strength resins utilized in the paper art can be found in TAPPI monograph series No. 29, Wet Strength in Paper and Paperboard, Technical Association of the Pulp and Paper Industry (N.Y., 1965). The most useful wet strength resins have generally been cationic in character. Polyamide-epichlorohydrin resins are cationic wet strength resins which have been found to be of particular utility. Suitable types of such resins are described in U.S. Pat. Nos. 3,700,623, issued on Oct. 24, 1972, and 3,772,076, issued on Nov. 13, 1973, both issued to Keim and both being hereby incorporated by reference. One commercial source of a useful polyamide-epichlorohydrin resins is Hercules, Inc. of Wilmington, Del., which markets such resin under the mark Kymene™ 557H.

Polyacrylamide resins have also been found to be of utility as wet strength resins. These resins are described in U.S. Pat. Nos. 3,556,932, issued on Jan. 19, 1971, to Coscia, et al. and 3,556,933, issued on Jan. 19, 1971, to Williams et al., both patents being incorporated herein by reference. One commercial source of polyacrylamide resins is American Cyanamid Co. of Stamford, Conn., which markets one such resin under the mark Parez™ 631NC.

Still other water-soluble cationic resins finding utility in this invention are urea formaldehyde and melamine formaldehyde resins. The more common functional groups of these polyfunctional resins are nitrogen containing groups such as amino groups and methylol groups attached to nitrogen. Polyethylenimine type resins may also find utility in the present invention. In addition, temporary wet strength resins such as Caldas 10 (manufactured by Japan Carlit) and CoBond 1000 (manufactured by National Starch and Chemical Company) may be used in the present invention. It is to be understood that the addition of chemical compounds such as the wet strength and temporary wet strength resins discussed above to the pulp furnish is optional and is not necessary for the practice of the present development.

The embryonic web 120 is preferably prepared from an aqueous dispersion of the papermaking fibers, though dispersions of the fibers in liquids other than water can be used. The fibers are dispersed in water to form an aqueous dispersion having a consistency of from about 0.1 to about 0.3 percent. The percent consistency of a dispersion, slurry, web, or other system is defined as 100 times the quotient obtained when the weight of dry fiber in the system under discussion is divided by the total weight of the system. Fiber weight is always expressed on the basis of bone dry fibers.

A second step in the practice of the present invention is forming the embryonic web 120 of papermaking fibers. Referring to FIG. 1, an aqueous dispersion of papermaking fibers is provided to a headbox 18 which can be of any convenient design. From the headbox 18 the aqueous dispersion of papermaking fibers is delivered to a foraminous forming member 11 to form an embryonic web 120. The forming member 11 can comprise a continuous Fourdrinier wire. Alternatively, the foraminous forming member 11 can comprise a plurality of polymeric protuberances joined to a continuous reinforcing structure to provide an embryonic web 120 having two or more distinct basis weight regions, such as is disclosed in U.S. Pat. No. 5,245,025 issued Sep. 14, 1993 to Trokhan et al., which patent is incorporated herein by reference. While a single forming member 11 is shown in FIG. 1, single or double wire forming apparatus may be used. Other forming wire configurations, such as S or C wrap configurations can be used.

The forming member 11 is supported by a breast roll 12 and a plurality of return rolls, of which only two return rolls 13 and 14 are shown in FIG. 1. The forming member 11 is driven in the direction indicated by the arrow 81 by a drive means not shown. The embryonic web 120 is formed from the aqueous dispersion of papermaking fibers by depositing the dispersion onto the foraminous forming member 11 and removing a portion of the aqueous dispersing medium. The embryonic web 120 has a first web face 122 contacting the foraminous member 11 and a second oppositely facing web face 124.

The embryonic web 120 can be formed in a continuous papermaking process, as shown in FIG. 1, or alternatively, a batch process, such as a handsheet making process can be used. After the aqueous dispersion of papermaking fibers is deposited onto the foraminous forming member 11, the embryonic web 120 is formed by removal of a portion of the aqueous dispersing medium by techniques well known to those skilled in the art. Vacuum boxes, forming boards, hydrofoils, and the like are useful in effecting water removal from the aqueous dispersion on the foraminous forming member 11. The embryonic web 120 travels with the forming member 11 about the return roll 13 and is brought into the proximity of a foraminous imprinting member 219.

The foraminous imprinting member 219 has a first web contacting face 220 and a second felt contacting face 240. The web contacting face 220 has a web imprinting surface 222 and a deflection conduit portion 230, as shown in FIGS. 2 and 3. The deflection conduit portion 230 forms at least a portion of a continuous passageway extending from the first face 220 to the second face 240 for carrying water through the foraminous imprinting member 219. Accordingly, when water is removed from the web of papermaking fibers in the direction of the foraminous imprinting member 219, the water can be disposed of without having to again contact the web of papermaking fibers. The foraminous imprinting member 219 can comprise an endless belt, as shown in FIG. 1, and can be supported by a plurality of rolls 201-217.

The foraminous imprinting member 219 is driven in the direction 281 (corresponding to the machine direction)

shown in FIG. 1 by a drive means (not shown). The first web contacting face 220 of the foraminous imprinting member 219 can be sprayed with an emulsion comprising about 90 percent by weight water, about 8 percent petroleum oil, about 1 percent cetyl alcohol, and about 1 percent of a surfactant such as Adogen TA-100. Such an emulsion facilitates transfer of the web from the imprinting member 219 to the drying drum 510. Of course, it will be understood that the foraminous imprinting member 219 need not comprise an endless belt if used in making handsheets in a batch process.

In the embodiment shown in FIGS. 2 and 3, the first web contacting face 220 of the foraminous imprinting member 219 comprises a macroscopically monoplanar, patterned, continuous network web imprinting surface 222. The continuous network web imprinting surface 222 defines within the foraminous imprinting member 219 a plurality of discrete, isolated, non-connecting deflection conduits 230. The deflection conduits 230 have openings 239 which can be random in shape and in distribution, but which are preferably of uniform shape and distributed in a repeating, preselected pattern on the first web contacting face 220. Such a continuous network web imprinting surface 222 and discrete deflection conduits 230 are useful for forming a paper structure having a continuous, relatively high density network region 1083 and a plurality of relatively low density domes 1084 dispersed throughout the continuous, relatively high density network region 1083, as shown in FIGS. 6 and 7.

Suitable shapes for the openings 239 include, but are not limited to, circles, ovals, and polygons, with hexagonal shaped openings 239 shown in FIG. 2. The openings 239 can be regularly and evenly spaced in aligned ranks and files. Alternatively, the openings 239 can be bilaterally staggered in the machine direction (MD) and cross-machine direction (CD), as shown in FIG. 2, where the machine direction refers to that direction which is parallel to the flow of the web through the equipment, and the cross machine direction is perpendicular to the machine direction. A foraminous imprinting member 219 having a continuous network web imprinting surface 222 and discrete isolated deflection conduits 230 can be manufactured according to the teachings of the following U.S. patents which are incorporated herein by reference: U.S. Pat. No. 4,514,345 issued Apr. 30, 1985 to Johnson et al.; U.S. Pat. No. 4,529,480 issued Jul. 16, 1985 to Trokhan; and U.S. Pat. No. 5,098,522 issued Mar. 24, 1992 to Smurkoski et al.; and U.S. Pat. No. 5,514,523 issued May 7, 1996 to Trokhan et al.

Referring to FIGS. 2 and 3, the foraminous imprinting member 219 can include a woven reinforcement element 243 for strengthening the foraminous imprinting member 219. The reinforcement element 243 can include machine direction reinforcing strands 242 and cross machine direction reinforcing strands 241, though any convenient weave pattern can be used. The openings in the woven reinforcement element 243 formed by the interstices between the stands 241 and 242 are smaller than the size of the openings 239 of the deflection conduits 230. Together, the openings in the woven reinforcement element 243 and the openings 239 of the deflection conduits 230 provide a continuous passageway extending from the first face 220 to the second face 240 for carrying water through the foraminous imprinting member 219. The reinforcement element 243 can also provide a support surface for limiting deflection of the fibers into the deflection conduits 230, and thereby help to prevent the formation of apertures in the portions of the web associated with the deflection conduits 230, such as the relatively low

density domes 1084. Such apertures, or pinholing, can be caused by water or air flow through the deflection conduits when a pressure difference exists across the web.

The area of the web imprinting surface 222, as a percentage of the total area of the first web contacting surface 220, should be between about 15 percent to about 65 percent, and more preferably between about 20 percent to about 50 percent to provide a desirable ratio of the areas of the relatively high density region 1083 and the relatively low density domes 1084 shown in FIGS. 6 and 7. The size of the openings 239 of the deflection conduits 230 in the plane of the first face 220 can be expressed in terms of effective free span. Effective free span is defined as the area of the opening 239 in the plane of the first face 220 divided by one fourth of the perimeter of the opening 239. The effective free span should be from about 0.25 to about 3.0 times the average length of the papermaking fibers used to form the embryonic web 120, and is preferably from about 0.5 to about 1.5 times the average length of the papermaking fibers. The deflection conduits 230 can have a depth 232 (FIG. 3) which is between about 0.1 mm and about 1.0 mm.

In an alternative embodiment, the foraminous imprinting member 219 can comprise a fabric belt formed of woven filaments. The web imprinting surface 222 can be formed by discrete knuckles formed at the cross-over points of the woven filaments. Suitable woven filament fabric belts for use as the foraminous imprinting member 219 are disclosed in U.S. Pat No. 3,301,746 issued Jan. 31, 1967 to Sanford et al., U.S. Pat. No. 3,905,863 issued Sep. 16, 1975 to Ayers, U.S. Pat. No. 4,191,609 issued Mar. 4, 1980 to Trokhan, and U.S. Pat. No. 4,239,065 issued Dec. 16, 1980 to Trokhan, which patents are incorporated herein by reference.

In another alternative embodiment, the foraminous imprinting member 219 can have a first web contacting face 220 comprising a continuous patterned deflection conduit 230 encompassing a plurality of discrete, isolated web imprinting surfaces 222. Such a foraminous imprinting member 219 can be used to form a molded web having a continuous, relatively low density network region, and a plurality of discrete, relatively high density regions dispersed throughout the continuous, relatively low density network. Such a foraminous imprinting member is shown in FIG. 11, as well as in U.S. Pat. No. 4,514,345 issued Apr. 30, 1985 to Johnson et al., which patent is incorporated herein by reference.

In yet another embodiment, the foraminous imprinting member 219 can have a first web contacting face 220 comprising a plurality of semicontinuous web imprinting surfaces 222. As used herein, a pattern of web imprinting surfaces 222 is considered to be semicontinuous if a plurality of the imprinting surfaces 222 extend substantially unbroken along any one direction on the web contacting face 220, and each imprinting surface is spaced apart from adjacent imprinting surfaces 220 by a deflection conduit 230. The web contacting face 220 can have adjacent semicontinuous imprinting surfaces 222 spaced apart by semicontinuous deflection conduits 230. The semicontinuous imprinting surfaces 222 can extend generally parallel to the machine or cross-machine directions, or alternatively, extend along a direction forming an angle with respect to the machine and cross-machine directions. Such a foraminous imprinting member is shown in FIG. 12, as well as in U.S. patent application Ser. No. 07/936,954, Papermaking Belt Having Semicontinuous Pattern and Paper Made Thereon, filed Aug. 26, 1992 in the name of Ayers et al., which applications is incorporated herein by reference.

A third step in the practice of the present invention comprises transferring the embryonic web 120 from the

foraminous forming member 11 to the foraminous imprinting member 219, to position the second web face 124 on the first web contacting face 220 of the foraminous imprinting member 219.

A fourth step in the practice of the present invention comprises deflecting a portion of the papermaking fibers in the embryonic web 120 into the deflection conduit portion 230 of web contacting face 220, and removing water from the embryonic web 120 through the deflection conduit portion 230 to form an intermediate web 120A of the papermaking fibers. The embryonic web 120 preferably has a consistency of between about 3 and about 20 percent at the point of transfer to facilitate deflection of the papermaking fibers into the deflection conduit portion 230.

The steps of transferring the embryonic web 120 to the imprinting member 219 and deflecting a portion of the papermaking fibers in the web 120 into the deflection conduit portion 230 can be provided, at least in part, by applying a differential fluid pressure to the embryonic web 120. For instance, the embryonic web 120 can be vacuum transferred from the forming member 11 to the imprinting member 219, such as by a vacuum box 126 shown in FIG. 1, or alternatively, by a rotary pickup vacuum roll (not shown). The pressure differential across the embryonic web 120 provided by the vacuum source (e.g., the vacuum box 126) deflects the fibers into the deflection conduit portion 230, and preferably removes water from the web through the deflection conduit portion 230 to raise the consistency of the web to between about 18 and about 30 percent. The pressure differential across the embryonic web 120 can be between about 13.5 kPa and about 40.6 kPa (between about 4 to about 12 inches of mercury). The vacuum provided by the vacuum box 126 permits transfer of the embryonic web 120 to the foraminous imprinting member 219 and deflection of the fibers into the deflection conduit portion 230 without compacting the embryonic web 120. Additional vacuum boxes can be included to further dewater the intermediate web 120A.

Referring to FIG. 4, portions of the intermediate web 120A are shown deflected into the deflection conduits 230 upstream of the compression nip 300, so that the intermediate web 120A is non-monoplanar. The intermediate web 120A is shown having a generally uniform thickness (distance between first and second web faces 122 and 124) upstream of the compression nip 300 to indicate that a portion of the intermediate web 120A has been deflected into the imprinting member 219 without locally densifying or compacting the intermediate web 120A upstream of the compression nip 300. Transfer of the embryonic web 120 and deflection of the fibers in the embryonic web into the deflection conduit portion 230 can be accomplished essentially simultaneously. Above referenced U.S. Pat. No. 4,529,480 is incorporated herein by reference for the purpose of teaching a method for transferring an embryonic web to a foraminous member and deflecting a portion of the papermaking fibers in the embryonic web into the foraminous member.

A fifth step in the practice of the present invention comprises pressing the wet intermediate web 120A in the compression nip 300 to form the molded web 120B. Referring to FIGS. 1 and 4, the intermediate web 120A is carried on the foraminous imprinting member 219 from the foraminous forming member 11 and through the compression nip 300 formed between the opposed compression surfaces of roll 362 and shoe press assembly 700. In order to describe the operation of the compression nip 300, the imprinting member 219, dewatering felts 320 and 360, and the paper web are drawn enlarged relative to the roll 362 and the press assembly 700.

The first dewatering felt 320 is shown supported in the compression nip adjacent the press shoe assembly 700, and is driven in the direction 321 around a plurality of felt support rolls 324. The shoe press assembly 700 includes a fluid impervious pressure belt 710, a pressure shoe 720, and pressure source P. The pressure shoe 720 can have a generally arcuate, concave surface 722. The pressure belt 710 travels in a continuous path over the generally concave surface 722 and the guide rolls 712. The pressure source P provides hydraulic fluid under pressure to a cavity (not shown) in the pressure shoe 720. The pressurized fluid in the cavity urges the pressure belt 710 against the felt 320, and provides the loading of the compression nip 300. Shoe press assemblies are disclosed generally in the following U.S. Patents, which are incorporated herein by reference: U.S. Pat. No. 4,559,258 to Kiuchi; U.S. Pat. No. 3,974,026 to Emson et al.; U.S. Pat. No. 4,287,021 to Justus et al.; U.S. Pat. No. 4,201,624 to Mohr et al.; U.S. Pat. No. 4,229,253 to Cronin; U.S. Pat. No. 4,561,939 to Justus; U.S. Pat. No. 5,389,205 to Pajula et al.; U.S. Pat. No. 5,178,732 to Steiner et al.; U.S. Pat. No. 5,308,450 to Braun et al.

The outer surface of the pressure belt 710 takes on a generally arcuate, concave shape as it passes over the pressure shoe 720, and provides a concave compression surface facing oppositely to the convex compression surface provided by press roll 362. This portion of the outer surface of the pressure belt 710 passing over the pressure shoe is designated 711 in FIG. 4. The outer surface of the pressure belt 710 can be smooth or grooved.

The convex compression surface provided by the press roll 362 in combination with the oppositely facing concave compression surface provided by the shoe press assembly 700 provide an arcuate compression nip having machine direction length which is at least about 3.0 inch. In one embodiment, the compression nip 300 has a machine direction length of between about 3.0 to about 20.0 inches, and more preferably between about 4.0 inches and about 10.0 inches.

The second dewatering felt 360 is shown supported in the compression nip 300 adjacent the nip roll 362 and driven in the direction 361 around a plurality of felt support rolls 364. A felt dewatering apparatus 370, such as a Uhle vacuum box can be associated with each of the dewatering felt 320 and 360 to remove water transferred to the dewatering felts from the intermediate web 120A.

The relatively high air permeability, open pore structure of the second felt 360 enhances the ability of the dewatering apparatus 370 to remove water from the felt 360. This ensures the felt 360 will not introduce water to the web at the entrance of the nip 300. In addition, the open pore structure of the felt 360 will also prevent water pressed from the web into the felt 360 (via the deflection conduits 230) from re-entering and rewetting the web at the exit of the nip felt 360.

The press roll 362 can have a generally smooth surface. Alternatively, the roll 362 can be grooved, or have a plurality of openings in flow communication with a source of vacuum for facilitating water removal from the intermediate web 120A. The roll 362 can have a rubber coating 363, such as a bonehard rubber cover, which can be smooth, grooved, or perforated. The rubber coating 363 shown in FIG. 4 provides a convex compression surface which face oppositely to the concave compression surface 711 provided by the shoe press assembly 700.

The term "dewatering felt" as used herein refers to a member which is absorbent, compressible, and flexible so

that it is deformable to follow the contour of the non-monoplanar intermediate web 120A on the imprinting member 219, and capable of receiving and containing water pressed from an intermediate web 120A. The dewatering felts 320 and 360 can be formed of natural materials, synthetic materials, or combinations thereof. A suitable dewatering felt layer comprises a nonwoven batt of natural or synthetic fibers joined, such as by needling, to a support structure formed of woven filaments. Suitable materials from which the nonwoven batt can be formed include but are not limited to natural fibers such as wool and synthetic fibers such as polyester and nylon. The fibers from which the batt 240 is formed can have a denier of between about 3 and about 40 grams per 9000 meters of filament length. The felt can have a layered construction, and comprise a mixture of fiber types and sizes.

The dewatering felt 320 can have a first surface 325 having a relatively high density, relatively small pore size, and a second surface 327 having a relatively low density, relatively large pore size. Likewise, the dewatering felt 360 can have a first surface 365 having a relatively high density, relatively small pore size, and a second surface 367 having a relatively low density, relatively large pore size.

The first dewatering felt 320 can have a thickness of between about 2 mm to about 5 mm, a basis weight of about 800 to about 2000 grams per square meter, an average density (basis weight divided by thickness) of between about 0.35 gram per cubic centimeter and about 0.45 gram per cubic centimeter.

The first felt 320 can have an air permeability of less than about 50 cubic feet per minute per square foot, at a pressure differential across the dewatering felt thickness of 0.12 kPa (0.5 inch of water). In one embodiment, the first felt 320 has an air permeability of between about 15 and about 25 cubic feet per minute per square foot. The air permeability is measured at a pressure difference of 0.5 inch of water, using a Valmet permeability measuring device (Model Wigo Taifun Type 1000 using Orifice #1) available from the Valmet Corp. of Pansio, Finland, or an equivalent device.

The first felt 320 can have a water holding capacity of at least about 150 milligrams of water per square centimeter of surface area, and a small pore capacity of at least about 100 milligrams per square centimeter. The water holding capacity is a measure of the amount of water held in pores having an effective radius between about 3 and about 500 micrometers in a one square centimeter section of the felt. The small pore capacity is a measure of the amount of water that can be contained in relatively small capillary openings in a one square centimeter section of a dewatering felt. By relatively small openings it is meant capillary openings having an effective radius of between about 3 to about 75 micrometers. Such capillary openings are similar in size to those in a wet paper web.

The water holding capacity and small pore capacity of a felt are measured using liquid porosimeter, such as a TRI Autoporosimeter available from TRI/Princeton Inc. of Princeton, N.J. The water holding capacity and small pore capacity are made according to a methodology described in U.S. patent application Ser. No. 08/461,832 "Web Patterning Apparatus Comprising a Felt Layer and a Photosensitive Resin Layer", filed Jun. 5, 1995 in the name of Trokhan et al., which patent application is incorporated herein by reference.

A suitable first dewatering felt 320 is an AmSeam-2, Style 2732 having a 1:1 batt to base ratio (1 pound batt material for every one pound of woven base reinforcing structure)

and a 3 over 6 layered batt construction (3 denier fibers over 6 denier fibers, where the 3 denier fibers are adjacent the surface **325** of the felt layer. Such a felt is available from Appleton Mills of Appleton, Wis. and can have an air permeability of about 25 cubic feet per minute per square foot.

The second dewatering felt **360** can have a thickness of between about 2 mm to about 5 mm, a basis weigh of about 800 to about 2000 grams per square meter, and an average density (basis weight divided by thickness) of between about 0.35 gram per cubic centimeter and about 0.45 gram per cubic centimeter.

The second felt **360** can have a water holding capacity which is less than that of the first felt **320**. The second felt **360** can also have a small pore capacity which is less than that of the first felt **320**. The second felt **360** can be a water holding capacity of less than about 150 milligrams of water per square centimeter of surface area, and a small pore capacity of less than about 100 milligrams per square centimeter.

The second felt **360** can have an air permeability of at least about 30 cubic feet per minute per square foot, and in one embodiment has an air permeability of at least about 40 cubic feet per minute per square foot. In one embodiment, the second felt **360** has an air permeability of between about 40 and about 120 cubic feet per minute per square foot.

A suitable second dewatering felt **360** is an AmFlex-3S Style 5615 having a 1:1 batt to base ratio and a 3 over 40 layered batt construction. Such a felt is available from Appleton Mills of Appleton, Wis. and can have an air permeability of about 40 cubic feet per minute per square foot.

The relatively high density and relatively small pore size of the first felt surfaces **325**, **365** promote rapid acquisition of the water pressed from the web in the nip **300**. The relatively low density and relatively large pore size of the second felt surfaces **327**, **367** provide space within the dewatering felts for storing water pressed from the web in the nip **300**.

The dewatering felts **320** and **360** can have a compressibility of between 20 and 80 percent, preferably between 30 and 70 percent, and more preferably between 40 and 60 percent. The "compressibility" as used herein is a measure of the percentage change in thickness of the dewatering felt under a given loading defined below. The dewatering felts **320** and **360** should also have a modulus of compression less than 10000 psi preferably less than 7000 psi, more preferably less than 5000 psi, and most preferably between about 1000 and about 4000 psi. The "modulus of compression" as used herein is a measure of the rate of change of loading with change in thickness of the dewatering felt. The compressibility and modulus of compression are measured using the following procedure. The dewatering felt is placed on a papermaking fabric formed of woven polyester monofilaments having a diameter of about 0.40 millimeter and having a square weave pattern of about 36 filaments per inch in a first direction, and about 30 filaments per inch in a second direction perpendicular to the first direction. The papermaking fabric has thickness under no compressive loading of about 0.68 millimeter (0.027 inch). Such a papermaking fabric is commercially available from the Appleton Wire Company of Appleton, Wis. The dewatering felt is positioned so that the surface of the dewatering felt which is normally in contact with the paper web is adjacent the papermaking fabric. The felt-fabric pair is then compressed with a constant rate tensile/compression tester, such as an

Instron Model 4502 available from the Instron Engineering Corporation of Canton, Mass. The tester has a circular compression foot having a surface of about 13 square centimeters (2.0 square inches) attached to a crosshead

5 moving at a rate of 5.08 centimeters per minute (2.0 inch per minute). The thickness of the felt-fabric pair is measured at loads of 0 psi, 300 psi, 450 psi, and 600 psi, where the load in psi is calculated by dividing the load in pounds obtained from the tester load cell by the surface area of the compression foot. The thickness of the fabric alone is also measured at 0 psi, 300 psi, 450 psi, and 600 psi loads. The compressibility and modulus of compression in psi are calculated using the following equations:

$$15 \text{ Compressibility} = 100 \times ((\text{TFPO} - \text{TPO}) - (\text{TFP450} - \text{TP450})) / (\text{TFPO} - \text{TPO})$$

$$10 \text{ Modulus of Compression} = (300 \text{ psi}) \times (\text{TFP300} - \text{TP300}) / ((\text{TFP300} - \text{TP300}) - (\text{TFP600} - \text{TP600}))$$

where TFPO, TFP300, TFP450, and TFP600 are the thicknesses of the felt-fabric pair at 0 psi, 300 psi, 450 psi and 600 psi loads, respectively, and TPO, TP300, TP450, and TP600 are the thicknesses of the fabric alone at 0 psi, 300 psi, 450 psi, and 600 psi loads, respectively.

The intermediate web **120A** and the web imprinting surface **222** are positioned intermediate the first and second felt layers **320** and **360** in the compression nip **300**. The first felt layer **320** is positioned adjacent the first face **122** of the intermediate web **120A**. The web imprinting surface **222** is positioned adjacent the second face **124** of the web **120A**. The second felt layer **360** is positioned in the compression nip **300** such that the second felt layer **360** is in flow communication with the deflection conduit portion **230**.

Referring to FIGS. 1 and 4, the first surface **325** of the first dewatering felt **320** is positioned adjacent the first face **122** of the intermediate web **120A** as the first dewatering felt **320** is driven over the belt **710**. Similarly, the first surface **365** of the second dewatering felt **360** is positioned adjacent the second felt contacting face **240** of the foraminous imprinting member **219** as the second dewatering felt **360** is driven around the nip roll **362**. Accordingly, as the intermediate web **120A** is carried through the compression nip **300** on the foraminous imprinting fabric **219**, the intermediate web **120A**, the imprinting fabric **219**, and the first and second dewatering felts **320** and **360** are pressed together between the opposed compression surfaces of the nip **300**. Pressing the intermediate web **120A** in the compression nip **300** further deflects the paper making fibers into the deflection conduit portion **230** of the imprinting member **219**, and removes water from the intermediate web **120A** to form the molded web **120B**. The water removed from the web is received by and contained in the dewatering felts **320** and **360**. Water is received by the dewatering felt **360** through the deflection conduit portion **230** of the imprinting member **219**.

55 The intermediate web **120A** should have a consistency of between about 14 and about 80 percent at the entrance to the compression nip **300**. More preferably, the intermediate web **120A** has a consistency between about 15 and about 35 percent at the entrance to the nip **300**. The papermaking fibers in an intermediate web **120A** having such a preferred consistency have relatively few fiber to fiber bonds, and can be relatively easily rearranged and deflected into the deflection conduit portion **230** by the first dewatering felt **320**.

60 The intermediate web **120A** is preferably pressed in the compression nip **300** at a nip pressure of at least 100 pounds per square inch (psi), and more preferably at least 200 psi. In a preferred embodiment, the intermediate web **120A** is

pressed in the compression nip **300** at a nip pressure greater than about 400 pounds per square inch.

The machine direction nip length can be between about 3.0 inches and about 20.0 inches. For a machine direction nip length between 4.0 inches to 10.0 inches, the press assembly **700** is preferably operated to provide between about 400 pounds of force per lineal inch of cross machine direction nip width and about 10000 pounds of force per lineal inch of cross machine direction nip width. The cross machine direction nip width is measured perpendicular to the plane of FIG. 4.

Pressing the web, felt layers, and imprinting member in a nip having a machine direction length of at least about 3.0 inches can improve dewatering of the web. For a given paper machine speed, the relatively long nip length increases the residence time of the web and the felts in the nip. Accordingly, water can be more effectively removed from the web, even at higher machine speeds.

The nip pressure in psi is calculated by dividing the nip force exerted on the web by the area of the nip **300**. The force exerted by the nip **300** is controlled by the pressure source *P*, and can be calculated using various force or pressure transducers familiar to those skilled in the art. The area of nip **300** is measured using a sheet of carbon paper and a sheet of plain white paper.

The carbon paper is placed on the sheet of plain paper. The carbon paper and the sheet of plain paper are placed in the compression nip **300** with the first and second dewatering felts **320**, **360** and the imprinting member **219**. The carbon paper is positioned adjacent the first dewatering felt **320** and the plain paper is positioned adjacent the imprinting member **219**. The shoe press assembly **700** is then activated to provide the desired press force, and the area of the nip **300** at that level of force is measured from the imprint that the carbon paper imparts to the sheet of plain white paper. Likewise, the machine direction nip length and the cross machine direction nip width can be determined from the imprint that the carbon paper imparts to the sheet of plain white paper.

The molded web **120B** is preferably pressed to have a consistency of at least about 30 percent at the exit of the compression nip **300**. Pressing the intermediate web **120A** as shown in FIG. 1 molds the web to provide a first relatively high density region **1083** associated with the web imprinting surface **222** and a second relatively low density region **1084** of the web associated with the deflection conduit portion **230**. Pressing the intermediate web **120A** on an imprinting fabric **219** having a macroscopically monoplanar, patterned, continuous network web imprinting surface **222**, as shown in FIGS. 2-4, provides a molded web **120B** having a macroscopically monoplanar, patterned, continuous network region **1083** having a relatively high density, and a plurality of discrete, relatively low density domes **1084** dispersed throughout the continuous, relatively high density network region **1083**. Such a molded web **120B** is shown in FIGS. 6 and 7. Such a molded web has the advantage that the continuous, relatively high density network region **1083** provides a continuous loadpath for carrying tensile loads.

The molded web **120B** is also characterized in having a third intermediate density region **1074** extending intermediate the first and second regions **1083** and **1084**, as shown in FIG. 8. The third region **1074** comprises a transition region **1073** positioned adjacent the first relatively high density region **1083**. The intermediate density region **1074** is formed as the first dewatering felt **320** draws papermaking fibers into the deflection conduit portion **230**, and has a tapered, generally trapezoidal cross-section.

The transition region **1073** is formed by compaction of the intermediate web **120A** at the perimeter of the deflection conduit portion **230**. The region **1073** encloses the intermediate density region **1074** to at least partially encircle each of the relatively low density domes **1084**. The transition region **1073** is characterized in having a thickness *T* which is a local minima, and which is less than the thickness *K* of the relatively high density region **1083**, and a local density which is greater than the density of the relatively high density region **1083**. The relatively low density domes **1084** have a thickness *P* which is a local maxima, and which is greater than the thickness *K* of the relatively high density, continuous network region **1083**. Without being limited by theory, it is believed that the transition region **1073** acts as a hinge which enhances web flexibility. The molded web **120B** formed by the process shown in FIG. 1 is characterized in having relatively high tensile strength and flexibility for a given level of web basis weight and web caliper *H* (FIG. 8).

The difference in density between the relatively high density region **1083** and the relatively low density region **1084** is provided, in part, by deflecting a portion of the embryonic web **120** into the deflection conduit portion **230** of the imprinting member **219** to provide a non-monoplanar intermediate web **120A** upstream of the compression nip **300**. A monoplanar web carried through the compression nip **300** would be subject to some uniform compaction, thereby increasing the minimum density in the molded web **120B**. The portions of the non-monoplanar intermediate web **120A** in the deflection conduit portion **230** avoid such uniform compaction, and therefore maintain a relatively low density.

The difference in density between the relatively high density region and the relatively low density region is also provided, in part, by pressing with both the first and second dewatering felts **320** and **360** to remove water from both faces of the web and prevent rewetting of the web. Water is expelled from the first and second web faces **122** and **124** as the intermediate web **120A** is pressed in the compression nip **300**. It is important that the water expelled from both faces of the web be removed from both faces of the web. Otherwise the expelled water can re-enter the molded web **120B** at the exit of the nip **300**. For instance, if the dewatering felt **360** is omitted, water expelled from the second web face **124** into the deflection conduit portion **230** can re-enter the molded web **120B** through the deflection conduit portion **230** of the imprinting member **219** at the exit of the nip **300**.

Re-entry of water into the molded web **120B** is undesirable because it decreases the consistency of the molded web **120B**, and reduces drying efficiency. In addition, re-entry of water into the molded web **120B** disrupts the fiber bonds formed during pressing of the intermediate web **120A** and de-densifies the web. In particular, water returning to the molded web **120B** will disrupt the bonds in the relatively high density region **1083**, and reduce the density and load carrying capability of that region. Water returning to the molded web **120B** can also disrupt the fiber bonds forming the transition region **1073**.

The dewatering felts **320** and **360** prevent rewetting of the molded web through both web faces **122** and **124**, and thereby help to maintain the relatively high density region **1083** and the transition region **1073**. In the embodiment shown in FIG. 1, the first dewatering felt **320** is preferably separated from the first face **122** of the molded web **120B** at the exit of the compression nip **300** to prevent water held in the dewatering felt **320** from rewetting the first face **122** of the web. As described above, conventional papermaking methods for pressing a web between two felts teach that the

web should follow the felt having the relatively high density and relatively lower pore size and air permeability. Applicants have found that in pressing a web with an imprinting member between two felt layers, improved dewatering can be obtained by the opposite of this conventional teaching. In particular, the Applicants have found that improved dewatering of the web can be obtained by using two felts with different air permeabilities, and removing the denser, relatively lower air permeability, finer pore felt from the web at the nip exit.

In the embodiment of FIG. 1, the second dewatering felt 360 is supported such that it is separated from the imprinting member 219 upstream of the nip and downstream of the nip. Alternatively, the second dewatering felt 360 can be positioned adjacent the imprinting member 219 upstream of the nip, downstream of the nip, or both upstream and downstream of the nip 300. The relatively high air permeability and relatively low density, large pore size of the second felt 360 permits water to be removed from the felt 360 effectively, regardless of whether the second felt 360 is positioned adjacent the imprinting member 219 upstream or downstream of the nip 300.

A sixth step in the practice of the present invention can comprise pre-drying the molded web 120B, such as with a through-air dryer 400 as shown in FIG. 1. The molded web 120B can be pre-dried by directing a drying gas, such as heated air, through the molded web 120B. In one embodiment, the heated air is directed first through the molded web 120B from the first web face 122 to the second web face 124, and subsequently through the deflection conduit portion 230 of the imprinting member 219 on which the molded web is carried. The air directed through the molded web 120B partially dries the molded web 120B. In addition, without being limited by theory, it is believed that air passing through the portion of the web associated with the deflection conduit portion 230 can further deflect the web into the deflection conduit portion 230, and reduce the density of the relatively low density region 1084, thereby increasing the bulk and apparent softness of the molded web 120B. In one embodiment the molded web 120B can have a consistency of between about 30 and about 65 percent upon entering the through air dryer 400, and a consistency of between about 40 and about 80 upon exiting the through air dryer 400.

Referring to FIG. 1, the through air dryer 400 can comprise a hollow rotating drum 410. The molded web 120B can be carried around the hollow drum 410 on the imprinting member 219, and heated air can be directed radially outward from the hollow drum 410 to pass through the web 120B and the imprinting member 219. Alternatively, the heated air can be directed radially inward (not shown). Suitable through air dryers for use in practicing the present invention are disclosed in U.S. Pat. No. 3,303,576 issued May 26, 1965 to Sisson and U.S. Pat. No. 5,274,930 issued Jan. 4, 1994 to Ensign et al., which patents are incorporated herein by reference. Alternatively, one or more through air dryers 400 or other suitable drying devices can be located upstream of the nip 300 to partially dry the web prior to pressing the web in the nip 300.

A seventh step in the practice of the present invention can comprise impressing the web imprinting surface 222 of the foraminous imprinting member 219 into the molded web 120B to form an imprinted web 120C. Impressing the web imprinting surface 222 into the molded web 120B serves to further densify the relatively high density region 1083 of the molded web, thereby increasing the difference in density between the regions 1083 and 1084. Referring to FIG. 1, the

molded web 120B is carried on the imprinting member 219 and interposed between the imprinting member 219 and an impression surface at a nip 490. The impression surface can comprise a surface 512 of a heated drying drum 510, and the nip 490 can be formed between a roll 209 and the dryer drum 510. The imprinted web 120C can then be adhered to the surface 512 of the dryer drum 510 with the aid of a creping adhesive, and finally dried. The dried, imprinted web 120C can be foreshortened as it is removed from the dryer drum 510, such as by creping the imprinted web 120C from the dryer drum with a doctor blade 524.

The method provided by the present invention is particularly useful for making paper webs having a basis weight of between about 10 grams per square meter to about 65 grams per square meter. Such paper webs are suitable for use in the manufacture of single and multiple ply tissue and paper towel products.

In an alternative embodiment of the present invention, the second felt 360 can be positioned adjacent the second face 240 of the imprinting member 219 as the molded web 120B is carried on the imprinting member 219 from the nip 300 to the nip 490. The nip 490 can be formed between a vacuum pressure roll and the Yankee drum 510.

An alternative embodiment of the present invention employs a composite imprinting member 219, and is illustrated in FIGS. 5, 9, and 10. Referring to FIG. 10, the composite imprinting member 219 has a web patterning photopolymer layer 221 joined to the surface 365 of a dewatering felt 360. The dewatering felt 360 comprises a nonwoven batt 3610 which can be needled to a support structure comprising woven filaments 3620.

The first dewatering felt 320 can be the above-mentioned AmSeam-2, Style 2732 having a 1:1 batt to base ratio, a 3 over 6 layered batt construction and an air permeability of about 25 cubic feet per minute per square foot.

The second dewatering felt 360 can be the above-mentioned AmFlex-3S Style 5615 having a 1:1 batt to base ratio, a 3 over 40 layered batt construction, and an air permeability of about 40 cubic feet per minute per square foot.

The photopolymer layer 221 has a macroscopically monoplanar, patterned continuous network web imprinting surface 222. Such a composite imprinting member 219 can comprise a photopolymer resin cast onto the surface of a dewatering felt. The following commonly assigned U.S. patent applications are incorporated herein by reference for the purpose of showing the construction of such a composite imprinting member: Ser. No. 08/461,832 "Web Patterning Apparatus Comprising a Felt Layer and a Photosensitive Resin Layer," filed Jun. 5, 1995 in the name of Trokhan, et al., which is a continuation in part of U.S. patent application Ser. No. 08/268,154 filed Jun. 29, 1994; U.S. Ser. No. 08/391,372 "Method of Applying a Curable Resin to a Substrate for Use in Papermaking" filed Feb. 15, 1995 in the name of Trokhan et al.; and "High Absorbence/Low Reflectance Felts with a Pattern Layer" filed Apr. 30, 1996 in the name of Ampulski et al.

In FIG. 9, the embryonic web 120 is transferred to the photopolymer web imprinting surface 222 of the composite imprinting member 219. The relatively high air permeability of the felt layer 360 facilitates transfer of the web to the composite imprinting member 219 by the vacuum box 126. The relatively high air permeability of the felt layer 360 also enhances water removal from the web at transfer. In addition, other vacuum operated dewatering equipment can be positioned intermediate the transfer point and the nip 300 to remove water from the felt 360 and web upstream of the

nip 300. For instance, a vacuum device 137 can be positioned adjacent to the composite imprinting member 219, as shown in FIG. 9, to remove water from the felt layer 360 and the web. The vacuum device 137 provides a vacuum which draws water from the web to the felt 360, and then from the felt 360 to the device 137. Suitable vacuum devices 137 include but are not limited to vacuum slots and vacuum pressure rolls.

The web is pressed in the nip 300 between the first felt 320 and the composite imprinting member 219, which comprises the photopolymer web imprinting surface 222 and the second felt 360. The deflection conduits 230 of the patterned photopolymer layer 221 are in flow communication with the felt layer 360, as shown in FIG. 10.

FIG. 5 is an enlarged illustration of the nip 300 shown in FIG. 9. The force provided by the shoe press assembly urges the felt 320 against the web 120A, causing discrete portions of the web 120A to be deflected into the deflection conduits 230, and compacting a continuous network portion of the web 120A, thereby forming a molded web 120B. At the exit of the nip 300, the felt 320 is removed from the molded web 120, and the molded web is carried on the composite imprinting member 219.

The molded web 120B is carried on the web imprinting surface 222 of the composite web imprinting member to the nip 490. The nip 490 in FIG. 9 is formed between a pressure roll 299 and the Yankee drum 510. The pressure roll 299 can be a vacuum pressure roll which removes water from the web via the second felt 360. The relatively high air permeability of felt 360 enhances this water removal. Alternatively, the pressure roll 299 can be a solid roll. With the composite imprinting member 219 positioned adjacent the face 124 of the molded web 120B, the web is carried on the composite imprinting member 219 into the nip 490 to transfer the molded web 120B to the Yankee drum 510.

While particular embodiments of the present invention have been illustrated and described, it would be obvious to those skilled in the art that various other changes and modifications can be made without departing from the spirit and scope of the present invention.

What is claimed:

1. A method of forming a fibrous web, the method comprising steps of:

(a) providing an embryonic fibrous web disposed on an imprinting member having a web contacting face and a felt contacting face opposite to the web contacting face, the web contacting face comprising a web imprinting surface and a deflection conduit portion, wherein the embryonic fibrous web is disposed on the web contacting face of the imprinting member;

(b) deflecting a first portion of the embryonic web into the deflection conduit portion, thereby forming an intermediate web, wherein a second portion of the intermediate web is associated with the web imprinting surface;

(c) providing a first dewatering felt layer and a second dewatering felt layer;

(d) providing a compression nip comprising a pair of mutually-opposed compression surfaces structured and configured to receive therebetween the first and second dewatering felt layers and the imprinting member having the intermediate fibrous web thereon;

(e) directing said imprinting member having the intermediate fibrous web thereon and the first and second felt layers through said compression nip such that the imprinting member and the web associated therewith are interposed between the first and second dewatering felt layers, wherein the first dewatering felt layer is adjacent to the web, and the deflection conduit portion of the imprinting member is in flow communication with the second dewatering felt layer; and

(f) pressing the imprinting member having the intermediate fibrous web disposed therein, and the first and second dewatering felt layers in the compression nip between said mutually-opposed compression surfaces, thereby further deflecting the first portion of the intermediate web into the deflection conduit portion and densifying the second portion of the intermediate web associated with the web imprinting surface.

2. The method according to claim 1, wherein the step of providing an embryonic web disposed on an imprinting member comprises:

providing an aqueous dispersion of papermaking fibers;  
providing a foraminous forming member;  
forming an embryonic web of the papermaking fibers on the foraminous forming member; and  
transferring the embryonic web from the foraminous forming member to the imprinting member.

3. The method of claim 2, wherein the step of transferring the embryonic web from the foraminous forming member to the imprinting member comprises vacuum transferring the embryonic web from the forming member to the imprinting member.

4. The method of claim 3, wherein the step of transferring the embryonic web comprises transferring the embryonic web to a composite imprinting member, and wherein the composite imprinting member comprises the second felt layer.

5. The method of claim 4, further comprising steps of:  
providing a vacuum device; and  
removing water from the second felt layer with the vacuum device intermediate the step of transferring the embryonic web to the composite imprinting member and the step of pressing the web in the compression nip.

6. The method of claim 5, comprising steps of:  
providing a composite imprinting member having a first web contacting face comprising a macroscopically monoplanar, patterned, continuous network web imprinting surface defining a plurality of discrete, isolated, non-connected deflection conduits; and  
pressing the web in the compression nip to form a molded web having a patterned continuous network region having a relatively high density, and a plurality of discrete domes having a relatively low density, the domes being dispersed throughout the continuous, relatively high density network region, and isolated one from another by the relatively high density network region.

7. The method of claim 1, wherein the second felt dewatering layer has an air permeability from about 30 to about 120 cubic feet per minute per square foot.

**21**

8. The method of claim 1, comprising steps of:  
providing an imprinting member having a first web contacting face comprising a macroscopically monoplanar, patterned, continuous network web imprinting surface defining a plurality of discrete, isolated, non-connected deflection conduits; and  
pressing the web in the compression nip to form a molded web having a patterned continuous network region having a relatively high density, and a plurality of discrete domes having a relatively low density, the domes being dispersed throughout the continuous, rela-

**22**

tively high density network region, and isolated one from another by the relatively high density network region.

9. The method of claim 1, wherein the first dewatering layer has an air permeability which is lower than an air permeability of the second dewatering felt layer.

10. The method of claim 1, wherein the first dewatering felt layer has a water holding capacity which is greater than a water holding capacity of the second dewatering felt layer.

\* \* \* \* \*